

## UNITED STATES PATENT OFFICE

2,133,848

## CORROSION RESISTANT TUBULAR ARTICLE

Donald K. Crampton, Marion, and Newell W. Mitchell, Waterbury, Conn., assignors to Chase Brass & Copper Co., Incorporated, Waterbury, Conn., a corporation

No Drawing. Application August 5, 1938,  
Serial No. 223,272

5 Claims. (Cl. 138—47)

This invention relates to improvements in corrosion-resistant tubular articles, and more particularly, corrosion-resistant wrought-metal tubular articles formed of copper-base alloys containing phosphorus, zinc and tin, with or without other elements which do not seriously impair the properties of the alloy.

This application is a continuation-in-part of our application Serial No. 71,807, filed March 30, 10 1936.

We have found that wrought-metal tubular articles, such, for example, as tubes, pipes, etc., made of copper-base alloys containing phosphorus from about  $\frac{1}{4}$  to about 2%, zinc from about 1% to about 30%, tin from about  $\frac{1}{2}\%$  to about 8%, and copper, the copper, phosphorus, zinc and tin constituting about 90% or more of the alloy, with or without one or more additional elements in such substantially-innocuous amounts as do not seriously impair the properties of the alloy, have valuable corrosion-resistant properties, especially when conveying or holding or otherwise contacting saline liquid or dilute acid. The additional elements may range up to 25 a total of about 10%, depending on what elements are added, some being more innocuous than others.

While each of the elements iron and antimony should not be present much in excess of about 30 0.1%, silver, which is comparatively innocuous, may be present to as high as about 10% provided not too much of other elements is present. Nickel may be present to as high as about 5%, and lead and silicon may each be present to as high 35 as about 3%.

We have discovered that arsenic has a particularly harmful effect on the corrosion resistance to saline liquid and dilute acid, of wrought-metal tubular articles made of copper-base alloys 40 herein set forth of copper, phosphorus, zinc and tin, even when the arsenic is present in very small amount. We have discovered it to be important that the tubular articles for use in contact with saline liquid or dilute acid and formed of these 45 copper-base alloys of copper, phosphorus, zinc and tin should be substantially free from arsenic, that is, that arsenic, if present at all, should not be present in excess of 0.1%. We have found that arsenic has a very harmful action which 50 brings about corrosion with consequent serious loss of tensile strength and ductility and ultimate destruction of the tubular article. Not only is this true when these articles are subjected to plain corrosion without stress in the presence of 55 saline liquid or dilute acid, but also when they

are subjected to mechanical stress in the presence of saline liquid or dilute acid. Under commercial conditions, the tubular articles are frequently used under mechanical stress while subjected to corrosion by saline liquid or dilute acid, the amount or rate of corrosion being accelerated by the mechanical stress. Failure by stress corrosion in actual service is a very serious problem. We have discovered that wrought-metal tubular articles formed from copper-base alloys herein 10 set forth of copper, phosphorus, zinc and tin, when substantially free of arsenic, have exceptional corrosion resistance to saline liquid and dilute acid, both when subjected to these fluids under conditions of mechanical stress and free of 15 stress.

Corrosion-resistant wrought-metal tubular articles in accordance with this invention are preferably formed of copper-base alloys of copper, phosphorus, zinc and tin without additional elements, although as previously explained, certain additional elements may be tolerated provided they are present only in such amounts as are 20 substantially innocuous.

Although the phosphorus may range from 25 about  $\frac{1}{4}\%$  to about 2%, the zinc from about 1% to 30 30%, and the tin from about  $\frac{1}{2}\%$  to about 8%, it is preferable to have the phosphorus from about  $\frac{1}{2}\%$  to about 1 $\frac{1}{2}\%$ , the zinc from about 3% to about 20%, and the tin from about 1 $\frac{1}{2}\%$  to about 5%. Within the ranges of the elements 35 of this preferred alloy range, three separate alloy types may advantageously be made, all having phosphorus from  $\frac{1}{2}\%$  to about 1 $\frac{1}{2}\%$ , the first having zinc from about 3% to about 7% with the tin from about 3% to about 5%, the second having zinc from about 7% to about 12% with the tin from about 2% to about 4%, and a third having zinc from about 12% to about 20% with the tin from about 1 $\frac{1}{2}\%$  to about 3%. And 40 within the ranges of said three alloy types, three alloys may be advantageously made having nominal composition as follows: all three have about 1% phosphorus, the first having about 5% zinc with about 4% tin, the second having about 45 10% zinc with about 3% tin, and the third having about 15% zinc with about 2% tin.

In all the corrosion-resistant wrought-metal tubular articles made in accordance with this invention, as the zinc content is increased from 50 about 1% to about 30%, it is preferable to decrease both the ratio of tin to phosphorus and the combined amounts of tin plus phosphorus.

The invention may be carried out in other 55 specific ways than those herein set forth without

departing from the spirit and essential characteristics of the invention, and the present embodiment are, therefore, to be considered in all respects as illustrative and not restrictive, and 5 all changes coming within the meaning and equivalency range of the appended claims are intended to be embraced therein.

We claim:

1. A wrought-metal tubular article for use in 10 contact with saline liquid or dilute acid and characterized by good corrosion resistance to saline liquid and dilute acid and formed from an alloy substantially free of arsenic and consisting of: phosphorus from about  $\frac{1}{4}\%$  to about 2%; zinc from about 1% to about 30%; tin from about  $\frac{1}{2}\%$  to about 8%; and the balance substantially of copper.
2. A wrought-metal tubular article for use in 15 contact with saline liquid or dilute acid and characterized by good corrosion resistance to saline liquid and dilute acid and formed from an alloy substantially free of arsenic and consisting of: phosphorus from about  $\frac{1}{2}\%$  to about  $1\frac{1}{2}\%$ ; zinc from about 3% to about 20%; tin from about  $1\frac{1}{2}\%$  to about 5%; and the balance substantially 20 of copper.
3. A wrought-metal tubular article for use in 25 contact with saline liquid or dilute acid and char-

acterized by good corrosion resistance to saline liquid and dilute acid and formed from an alloy substantially free of arsenic and consisting of: phosphorus from about  $\frac{1}{2}\%$  to about  $1\frac{1}{2}\%$ ; zinc from about 3% to about 7%; tin from about 3% to about 5%; and the balance substantially of copper.

4. A wrought-metal tubular article for use in 5 contact with saline liquid or dilute acid and characterized by good corrosion resistance to 10 saline liquid and dilute acid and formed from an alloy substantially free of arsenic and consisting of: phosphorus from about  $\frac{1}{2}\%$  to about  $1\frac{1}{2}\%$ ; zinc from about 7% to about 12%; tin from about 2% to about 4%; and the balance substantially 15 of copper.

5. A wrought-metal tubular article for use in 20 contact with saline liquid or dilute acid and characterized by good corrosion resistance to saline liquid and dilute acid and formed from an alloy 25 substantially free of arsenic and consisting of: phosphorus from about  $\frac{1}{2}\%$  to about  $1\frac{1}{2}\%$ ; zinc from about 12% to about 20%; tin from about  $1\frac{1}{2}\%$  to about 3%; and the balance substantially of copper.

DONALD K. CRAMPTON.  
N. W. MITCHELL.